

## UNITED STATES PATENT OFFICE

FRANK C. HOFFMAN, OF SOUTH AMBOY, NEW JERSEY, ASSIGNOR TO E. I. DU PONT DE NEMOURS & COMPANY, OF WILMINGTON, DELAWARE, A CORPORATION OF DELAWARE

## PYROXYLIN ENAMEL

No Drawing.

Application filed August 28, 1928. Serial No. 302,643.

This invention relates to coating compositions and more particularly it relates to a special composition to be added to pyroxylin enamels to modify their usual characteristics on drying.

The usual type of pyroxylin enamel, when applied to a surface to be coated, dries rapidly to produce a continuous, tough, opaque surface. In order to simulate the effect of natural aging and cracking, enamels known as crackle enamels have been developed. These are lacquer enamels in which the pigment content is so great that it cannot be kept together by the lacquer binder with the result that when they are applied by spraying or otherwise to a lacquer ground coat, they split apart in irregular cracks, showing the color of the ground coat underneath. The finish thus produced has an aged, cracked or checked appearance. Heretofore, crackle enamels have been produced by compounding the desired ingredients according to a variety of formulas. The enamels thus produced accordingly made up a special class of products and it has been necessary for those handling these materials in stock to carry a double line of enamels, one consisting of ordinary enamels and the other consisting of a line of specially compounded crackle enamels.

This invention has as an object to provide a special product or ingredient which may be added to any of the usual types of pyroxylin enamels to modify their usual characteristics on drying. A further object is to make possible the conversion of the ordinary pyroxylin enamels into crackle enamels by the simple operation of mixing a single ingredient therewith. Other objects will appear hereinafter.

These objects are accomplished by the following invention which includes mixing a finely divided soap with a nitrocellulose solvent or thinner.

Throughout this specification for the purpose of more particularly describing the character of my special product, I shall refer to it as a "crackle base."

In carrying out this invention, a metallic soap, such for example, as an aluminum soap, is mixed with a solvent such as ethyl acetate. The mixture is then ground in a porcelain-

lined mill, using flint pebbles as the grinder. It is to be understood, of course, that the method of grinding which may be employed is not limited to the use of a pebble mill, but that other grinding methods may be used, provided the soap is properly ground and is not greatly discolored. In the grinding operation, a small quantity of pyroxylin may be added, if desired, in order to give body to the grinding mixture. The pyroxylin may be omitted altogether, however, since it is merely accessory to the compounding of the special ingredient of this invention.

The proportions of materials used may be varied within wide limits, but the following example is given as illustrating the proportions used in one of the preferred embodiments of my invention.

| Example           | Per cent |
|-------------------|----------|
| Aluminum stearate | 70       |
| Ethyl acetate     | 25       |
| Pyroxylin         | .5       |
|                   | 100      |
|                   | 75       |

In the example given above, the solvent may be substituted by other solvents than ethyl acetate capable of dissolving pyroxylin, but it should be carefully selected in order that the qualities of the crackle base will be preserved during storage. All solvents or thinners may not be used for making the crackle base of my invention, and it is to be noted that hydrocarbons are not suitable for this purpose, as they have a tendency to cause the base to gel during storage. Any of the aliphatic alcohols and esters may be used as a solvent in the formulation with satisfactory results.

It is to be understood that it is within the scope of my invention to use other soaps than aluminum stearate in compounding my crackle base. For instance, soaps formed by the interaction of other metals than those of aluminum with other fatty acids than stearic may be substituted for all or a part of the aluminum stearate given in the example, if desired.

In using the crackle base of my invention,

the proportions by weight of this material to the pyroxylin enamel to which it is added varies from 60% to 40%. However, these proportions are flexible and may be varied 5 to suit the particular type of enamel with which it is desired to mix the base. When thinning the mixture of enamel and crackle base, it is desirable to use ethyl acetate or some other readily volatile solvent in order 10 to hasten the drying speed.

It will thus be seen that I have provided a special product which makes it possible easily and quickly to convert the ordinary 15 types of pyroxylin enamels to the type known as crackle enamels. This eliminates the necessity, which has heretofore existed, of dealers in these enamels carrying a double line of materials. All that is now necessary is to stock the usual line of enamels and a 20 quantity of the special crackle base of my invention. When it is desired to produce a crackle finish with any of the usual types of enamels, they may be combined with the crackle base in the proportions indicated by 25 the character of the enamel. The crackle base has a low tinting strength and does not materially change the color of the enamel to which it is added.

As many apparently widely different 30 embodiments of this invention may be made without departing from the spirit thereof, it is to be understood that I do not limit myself to the foregoing examples or description except as indicated in the following patent 35 claims.

I claim:

1. The method of producing a coating 40 composition that will produce a crackle finish comprising adding to a completed cellulose nitrate coating composition a second composition comprising finely divided soap suspended in a cellulose nitrate solvent from the group consisting of aliphatic alcohols and esters, the second composition being added 45 in such amount that the soap in the final composition is between 10% to 15% by weight of the first composition.

2. The method of producing a coating 50 composition that will produce a crackle finish comprising adding to a completed cellulose nitrate composition a second composition comprising finely divided aluminum stearate suspended in a cellulose nitrate solvent from a group consisting of aliphatic alcohols and 55 esters, the second composition being added in such amount that the aluminum stearate in the final composition is between 10% to 15% by weight of the first composition.

3. The method of producing a coating 60 composition that will produce a crackle finish comprising adding to a completed cellulose nitrate coating composition a second composition comprising finely divided aluminum stearate, cellulose nitrate, and a cellulose nitrate solvent from the group consisting of 65

aliphatic alcohols and esters, the second composition being added in such amount that the aluminum stearate in the final composition is between 10% and 15% by weight of the first composition.

4. The method of producing a coating composition that will produce a crackle finish comprising adding to a completed cellulose nitrate coating composition a second composition comprising finely divided aluminum 70 stearate suspended in ethyl acetate, the second composition being added in such amount that the aluminum stearate in the final composition is between 10% to 15% by weight of the first composition.

5. The method of producing a coating composition that will produce a crackle finish comprising adding to a completed cellulose nitrate coating composition from 40% to 60% by weight thereof of a composition comprising approximately by weight 25% aluminum stearate, 74.5% ethyl acetate and 0.5% cellulose nitrate.

In testimony whereof, I affix my signature.

FRANK C. HOFFMAN.

90

95

100

105

110

115

120

125

130